

1

3,454,159

## PHOSPHATE FLOTATION

Clinton A. Hollingsworth, Lakeland, and Bobby L. Sapp, Plant City, Fla., assignors to Borden, Inc., New York, N.Y., a corporation of New Jersey  
No Drawing. Filed Apr. 21, 1966, Ser. No. 544,090  
Int. Cl. B03d 1/06

U.S. Cl. 209—3

5 Claims

## ABSTRACT OF THE DISCLOSURE

A method of beneficiating phosphate rock by anionic froth flotation by scrubbing a deslimed phosphate rock feed with an alkaline composition, dewatering and desliming the scrubbed feed, conditioning the thus treated feed with an anionic flotation reagent and subjecting the conditioned feed to a froth flotation of high grade phosphate concentrate.

This invention relates to the beneficiation of phosphate rock and similar phosphatic materials and in particular to an improved method of treating phosphate rock flotation feed to obtain a high grade phosphate concentrate.

In the usual process for beneficiating such phosphate-containing material (hereinafter referred to collectively as phosphate rock), the mixture of phosphatic minerals and gangue obtained from the phosphate deposit or mine is first washed to remove trash therefrom and to separate and recover the larger lumps of phosphate minerals (usually referred to as pebble rock). The remaining material (washer reject material) consists of a mixture of phosphate rock particles, sand, clay and similar gangue materials, substantially all of which is less than about 10 mesh (Tyler Standard), and preferably is less than 14 mesh in size. The phosphate rock constituent of this material is then concentrated and recovered for subsequent use, commonly by froth or table flotation techniques or a combination of both. Patents No. 3,013,664 and 3,086,654 to Hollingsworth and Sapp disclose efficient and economical methods of beneficiation utilizing froth flotation operations comprising cationic (silica) floats and anionic (phosphate) floats. At present, most flotation processes use a anionic float followed by a cationic float.

In such anionic flotation operations the phosphate rock feed is commonly first deslimed and dewatered, conditioned with an anionic flotation reagent, and subjected to a froth flotation operation, all as described in the Hollingsworth and Sapp patents noted above. In conventional practice the phosphate rock feed is sometimes scrubbed, as a slurry with water, prior to desliming and dewatering to aid in removal of adherent materials.

While superior to previous methods, the anionic flotation operation is not entirely satisfactory in that large quantities of anionic flotation reagents are consumed adding to the cost of beneficiation. Equally important, the flotation is not selective enough, resulting in a significant proportion of insolubles (mostly silica) being separated along with the phosphate.

A method has now been found whereby the amount of anionic flotation reagents required for effective flotation is greatly reduced, while at the same time the selectivity of the float is increased.

Briefly stated, the present invention comprises the method of beneficiating phosphate rock by froth flotation comprising scrubbing a phosphate rock feed with an alkaline

2

composition, conditioning the scrubbed rock feed with an anionic flotation reagent consisting essentially of a fatty acid and a fuel oil, and subjecting the conditioned feed to a froth flotation operation to float a final phosphate concentrate which is recovered as the desired phosphate product. In its preferred embodiment, the process also comprises dewatering and desliming the scrubbed phosphate rock feed prior to conditioning.

As to materials, the alkaline composition is preferably an aqueous solution of caustic soda. Other alkaline materials that may be used are soda ash, lime, ammonia, potassium hydroxide, magnesium hydroxide, and the like alkaline materials capable of raising the pH of an aqueous solution to at least about 8 and preferably about 9 and above. It is commercially uneconomical to use a pH above 11 because of the amount of alkaline material required. As to the proportions, the alkaline material is present in the scrubbing fluid in amount sufficient to adjust the pH of the fluid to about 9 and preferably 10. When caustic soda (NaOH) is the alkaline material to be added to the feed scrubbing step (scrubbing ordinarily is carried out at 65%—70% solids) it is used in the proportion of from about 0.005 part to about 0.05 part by weight for each 100 parts weight of phosphate rock feed.

The anionic flotation reagent is a combination of a fatty acid and a fuel oil. No alkaline materials are required as part of the reagent as is the case with anionic flotation reagent combination used heretofore in flotation of Florida phosphate rock feeds. The fatty acid may be oleic acid, linoleic acid, tall oils, rosin, mixtures thereof, and other like materials commonly used in anionic flotation reagents. In like manner, the fuel oil can be any commonly employed in anionic flotation reagents such as diesel oil, kerosene, Bunker C fuel oil, and mixtures thereof. The reagent is preferably a combination of 4 parts by weight of a fuel oil to each part by weight of a fatty acid, although proportions ranging from 1:1 to 8:1 can be used.

As to equipment the dewaterer, desliming, conditioner, and flotation apparatus can be those disclosed in the Hollingsworth and Sapp patents discussed above or those commonly used in phosphate beneficiation. The scrubber is preferably a standard attrition type scrubber.

As to processing conditions, a phosphate rock feed is first passed into a scrubber where it is scrubbed with the alkaline composition for time sufficient to render the surface of the phosphate rock sufficiently alkaline; ordinarily about 20 to about 60 seconds are required for small scale operations and up to about 3 minutes in large commercial installation. Longer treatment times can be used, but, again, this is not commercially desirable. The treatment time will vary, dependent upon the type of scrubbing equipment, the type and concentration of alkaline material in the scrubbing liquid. The optimum conditions are readily determinable by making test runs and noting the conditions showing the least amount of reagent used and the greatest recovery of phosphate. Phosphate recovery is measured as percent by weight of bone phosphate of lime (tricalcium phosphate) recovered or percent B.P.L. recovered. Using an amount of caustic soda in the scrubber solution to give a pH of about 10, it is found that treatment of phosphate rock feed for about 60 seconds will result in greatest percent B.P.L. recovery and lowest reagent consumption. If the feed has not been first subjected to a cationic flotation it should be deslimed prior to scrubbing.

After scrubbing, it is preferred to deslime and dewater the phosphate rock feed to remove slime produced in the scrubbing operation. Slime, either phosphatic or clay, if present in any appreciable amount, act to lower the effectiveness of the anionic flotation.

The phosphate rock feed is then conditioned by being admixed with an anionic flotation reagent of the present invention. The examples set forth below show that the instant invention requires less of the costly anionic flotation reagents components (fatty acid and fuel oil) than that required previously. More particularly, with 30 to 40% less anionic flotation reagent there is an increase in selectivity (less insolubles) while maintaining the same or better B.P.L. recovery.

The invention will be further described in connection with the following examples of the practice of it which are set forth for purposes of illustration only.

to eliminate variations due to equipment differences. The amount of alkaline material used in scrubbing and amount of anionic reagent used are measured in pounds per long ton of phosphate rock feed.

#### Example 1

The process of the present invention was compared with conventional procedures using a 29.72% B.P.L. phosphate rock feed. The feed was scrubbed in a series of runs, with and without caustic soda, for various periods of time at 65% solids using a turbo-type mixer. The several scrubbed feeds were then deslimed and conditioned with varying amounts of anionic flotation reagents containing 4 parts by weight of fuel oil to 1 part by weight of fatty acid and floated in a standard flotation cell. The fuel oil used was Bunker C fuel oil API gravity 19-20 and the fatty acid was Unitol OT (a tall oil fraction). The results are summarized in Table 1.

5  
10  
15

## Example 3

The process of the present invention was compared to conventional anionic floats employing no scrubbing and conventional anionic floats utilizing scrubbing. The other processing conditions used were the same as that used in Example 1. The results are summarized in Table 3.

3. The method according to claim 2 in which the alkaline material is used in an amount sufficient to adjust the pH of the solution to at least about 8.

4. The method according to claim 1 in which the phosphate rock feed is scrubbed with the alkaline composition for about 20 second to about 3 minutes.

TABLE 3

| Run No.                           | NaOH/<br>T.F. | pH    | Feed,<br>B.P.L. | Concentrate    |                  | Middling       |        | Tailing        |        | Percent<br>B.P.L.<br>Recy. | Lbs. Reagent/T.F. |      |     |      |     |
|-----------------------------------|---------------|-------|-----------------|----------------|------------------|----------------|--------|----------------|--------|----------------------------|-------------------|------|-----|------|-----|
|                                   |               |       |                 | Percent<br>Wt. | B.P.L.<br>Insol. | Percent<br>Wt. | B.P.L. | Percent<br>Wt. | B.P.L. |                            | 4:1<br>Mix        | NaOH | pH  |      |     |
| Standard Phosphate Floats         |               |       |                 |                |                  |                |        |                |        |                            |                   |      |     |      |     |
| 24.....                           | 36.66         | 9.7   | 80.55           | 1.46           | 15.7             | 74.18          | 74.6   | 22.17          | 4.03   | 54.5                       | 5.4               | .3   | 9.5 |      |     |
| 25.....                           | 36.66         | 37.6  | 79.05           | 3.68           | 3.8              | 37.42          | 58.6   | 9.52           | 2.56   | 84.2                       | 7.6               | .3   | 9.0 |      |     |
| 26.....                           | 36.66         | 37.6  | 78.38           | 4.33           | 4.4              | 35.42          | 58.0   | 9.85           | 2.55   | 83.8                       | 8.8               | .3   | 9.0 |      |     |
| 27.....                           | 36.66         | 39.5  | 78.28           | 4.55           | 4.5              | 29.67          | 56.0   | 8.64           | 2.49   | 85.8                       | 8.8               | .3   | 9.2 |      |     |
| 30 Sec. Scrubbing Without Caustic |               |       |                 |                |                  |                |        |                |        |                            |                   |      |     |      |     |
| 28.....                           | 7.2           | 36.66 | 25.3            | 79.67          | 2.02             | 8.9            | 64.55  | 65.8           | 15.14  | 2.99                       | 72.6              | 5.4  | .3  | 10   |     |
| 29.....                           | 7.2           | 36.66 | 39.2            | 76.71          | 5.58             | 3.2            | 19.86  | 57.6           | 10.75  | 2.55                       | 82.1              | 6.6  | .3  | 9.2  |     |
| 30.....                           | 7.2           | 36.66 | 41.5            | 77.70          | 4.63             | 4.1            | 26.23  | 54.4           | 8.78   | 2.47                       | 85.8              | 8.8  | .3  | 9.2  |     |
| 30 Sec. Scrubbing With Caustic    |               |       |                 |                |                  |                |        |                |        |                            |                   |      |     |      |     |
| 31.....                           | 3             | 10    | 36.66           | 41.5           | 77.43            | 4.66           | 3.5    | 21.95          | 55.0   | 6.58                       | 2.36              | 89.6 | 6.2 | None | 9.2 |
| 32.....                           | 3             | 10    | 36.66           | 40.7           | 78.46            | 3.56           | 3.5    | 32.04          | 55.8   | 6.26                       | 2.37              | 90.3 | 5.8 | None | 9.2 |

While the exact theory is not precisely understood, it is believed that scrubbing of the phosphate ore in the presence of an alkaline material prior to conditioning acts to clean the surface of the ore and to make the surface more alkaline or positive. This more positive charge on the clean surface, in turn, renders the separation in the anionic float more definite, greatly reducing the amount of insolubles separated with the phosphate and requiring much less anionic flotation reagent for effective flotation.

The anionic floatation procedure of the present invention can be used alone to beneficiate washer reject material or in conjunction with cationic floats carried out prior to or subsequent to the anionic floatation.

The scrubbing with alkaline material is also beneficial for cationic (silica) floatation as it acts to reduce the amount of reagent necessary while maintaining the same or better B.P.L. recovery.

What is claimed is:

1. The method of beneficiating phosphate rock by froth floatation comprising scrubbing a deslimed phosphate rock feed with an alkaline composition, dewatering and desliming the scrubbed feed to remove slime formed during scrubbing, conditioning the phosphate rock feed with an anionic floatation reagent consisting essentially of a fatty acid and a fuel oil, and subjecting the conditioned feed to a froth floatation operation to float a final phosphate concentrate which is recovered as the desired phosphate product.

2. The method according to claim 1 in which the alkaline composition is caustic soda.

30 5. The method of beneficiating phosphate rock by anionic froth floatation comprising scrubbing a deslimed phosphate rock feed with an aqueous solution of caustic soda of about pH 8 or above for about 20 seconds to about 3 minutes, dewatering and desliming the scrubbed feed to remove slime formed during scrubbing, conditioning the dewatered and deslimed feed with an anionic floatation reagent consisting essentially of a fuel oil and a fatty acid, and subjecting the conditioned feed to a froth floatation operation to float a phosphate concentrate which is recovered as the desired phosphate product.

## 40 References Cited

## UNITED STATES PATENTS

|           |         |          |           |
|-----------|---------|----------|-----------|
| 2,313,360 | 3/1943  | Ralston  | 209—166   |
| 2,336,437 | 12/1943 | Erickson | 209—166   |
| 2,424,552 | 7/1947  | Clemmer  | 209—166   |
| 2,660,303 | 11/1953 | Maseman  | 209—5     |
| 3,302,785 | 2/1967  | Greene   | 209—5     |
| 3,349,903 | 10/1967 | Olsen    | 209—166 X |

## 50 OTHER REFERENCES

50 Taggart, handbook of Mineral Dressing, Wiley and Sons, Inc., New York, 1945, 3-15, 3-17, 10-01, 10-07, TN 500 T3, 1945.

HARRY B. THORNTON, Primary Examiner.

55 R. HALPER, Assistant Examiner.

U.S. Cl. X.R.

209—12, 166